

July 10, 1945.

M. D. McINTOSH

2,379,915

MEDIA FOR USE IN MAKING CAMERA COPY AND METHODS OF PREPARING SAME

Filed July 30, 1942

2 Sheets-Sheet 1



FIG. 1.



FIG. 4.



FIG. 2.



FIG. 5.



FIG. 3.

INVENTOR.  
MAURICE D. McINTOSH.

BY *Gray, Macklin, Golick*  
*Williams, Chilton and Adler.*  
ATTORNEYS.

July 10, 1945.

M. D. MCINTOSH

2,379,915

MEDIA FOR USE IN MAKING CAMERA COPY AND METHODS OF PREPARING SAME

Filed July 30, 1942

2 Sheets-Sheet 2



FIG. 6.



FIG. 9.



FIG. 7.



FIG. 10.



FIG. 8.

INVENTOR.  
MAURICE D. MCINTOSH  
BY  
*Fay, Macklin, Golnick*  
*Williams, Hilton and Deller*  
ATTORNEYS.

Patented July 10, 1945

2,379,915

# UNITED STATES PATENT OFFICE

2,379,915

## MEDIA FOR USE IN MAKING CAMERA COPY AND METHOD OF PREPARING SAME

Maurice D. McIntosh, Cleveland Heights, Ohio,  
assignor to Louis S. Sanders, Shaker Heights,  
Ohio

Application July 30, 1942, Serial No. 452,863

10 Claims. (Cl. 41—41)

This invention relates, as indicated, to media for use in making camera copy, and to methods of preparing the same.

In my Reissue Patent No. 20,503, I have described a drawing paper having a plurality of normally invisible patterns, one of the patterns being developable by a developer solution capable of developing said pattern only and both of the patterns being developable by a developer solution capable of developing both of the patterns collectively. In the specific example described in said patent, one of the patterns consists of a plurality of geometrically arranged dots located in equally-spaced diagonal rows in such a manner that the dots in one of the rows align with adjacent dots in the other rows to form diagonal rows extending transversely of the first-named rows. The other pattern consists of diagonal lines extending longitudinally of and in registry with the respective diagonal rows of dots.

While this method of forming the patterns is, in general, satisfactory, its value depends to a great extent on securing perfect registry or proper relative location between the dots and lines, a condition which is often exceedingly difficult to obtain by the ordinary method of forming the patterns, that is, printing the patterns by means of plates.

I have discovered, however, that I can secure perfect registry or proper relative location between two different patterns by the simple expedient of printing on a suitable sheet or surface two sets of closely spaced parallel lines of chemically developable material, one set of lines crossing or intersecting the other set of lines at an angle of 90 degrees. In this way, I have been able to provide a medium which is not only useful for general drawing purposes, but which is especially adapted for use in the preparation of camera copy for multicolor printing.

The invention can probably best be understood by reference to the accompanying drawings, wherein

Fig. 1 is a plan view of a fragment or corner portion of a base sheet, illustrating the first imprint thereon;

Fig. 2 is a view similar to Fig. 1, but showing the second imprint as well as the first;

Fig. 3 is a view similar to Fig. 2, but showing the sheet after removal of the soluble portions of the lines forming the second imprint;

Fig. 4 is a view of the sheet as shown in Fig. 3, after development of the mercurous chloride pattern;

Fig. 5 is a view of the sheet as shown in Fig. 3, after development of both the mercurous chloride and basic lead sulphate patterns;

Fig. 6 is a view similar to Fig. 1, but illustrat-

ing the first imprint in the preparation of a modified form of the medium of the invention;

Fig. 7 is a view similar to Fig. 6, but illustrating the second imprint, as well as the first;

Fig. 8 is a view of the sheet removal of the varnish lines;

Fig. 9 is a view of the sheet, after development of the mercurous chloride pattern, and

Fig. 10 is a view of the sheet, after development of the mercurous chloride and lead sulphate squares.

Referring more particularly to Figs. 1 to 5 of the drawings, I first take a sheet of paper, cellulose acetate or nitrate film, ethyl cellulose film or similar material, which I have designated by reference numeral 2 in Fig. 1 of the drawings, and the surface of which is smooth, relatively impermeable to water and offers poor adhesion to glue. Sheets of cellulose acetate, cellulose nitrate and ethyl cellulose, in the condition in which they are usually available in the market, are satisfactory. Where, however, it is desired to use paper as a base, it is necessary to adhesively secure one of the foregoing cellulose sheets to the paper so as to provide a suitable surface, or to coat such paper with any one of a number of available waterproof lacquers, varnishes or synthetic resins.

For the purpose of the present description, it will be assumed that paper coated with a thin sheet 2 of cellulose acetate is used as the base of the drawing medium.

Using an ordinary printing plate bearing a parallel line pattern, in which the lines are as wide as the spaces between them, the first imprint consisting of such lines, designated 3, is printed. This imprint is made with ordinary white printing ink or clear printing varnish, applied directly to the acetate. Before the ink or varnish is dry and while it is still tacky, it is dusted with basic lead sulphate, a fine white powder. Various mechanical methods may be employed to dust the ink or varnish pattern, but it is not only necessary to bring the powder in contact with the tacky ink or varnish to have it adhere sufficiently to cover the whole ink or varnish surface. The dusted ink or varnish is then permitted to dry and firmly hold the powder embedded in its upper surface.

The entire surface of the sheet is then sponged gently under a spray of water to remove all excess and unbound or unembedded powder. The sheet is then dried by running it through soft rubber rollers, blotting, or other means, and is then ready to receive the second imprint.

The second imprint, consisting of the lines 4 shown in Fig. 2, is made with a printing plate identical with that used for making the first imprint, but the lines of which extend transversely

of or at 90 degrees to those of the first plate. This second imprint is made with an ink of the following composition, and treated in the following manner:

|                                                     | Parts |
|-----------------------------------------------------|-------|
| Liquid glue (Le Page's)                             | 120   |
| Glycerol                                            | 60    |
| Light blue watercolor solution (Eastman's<br>Velox) | 35    |
| Water (distilled)                                   | 300   |
| Mercurous chloride (precipitated powder)            | 900   |

After this ink has been ground on a stone paint mill several times or until the mercurous chloride powder is completely and very finely dispersed, 230 parts of diethylene glycol are added.

This ink is normally soluble in water, even when dry, but when imprinted as lines across the first imprint of dusted varnish lines, it penetrates the dusted lines at the points of superimposition and becomes insoluble, while the portions of the lines of soluble ink that fall on the cellulose acetate surface between the varnish lines remain soluble and removable.

This second print is permitted to dry and the sheet is then sponged under a spray of water until all soluble portions are removed. This leaves the insoluble portions superimposed on the dusted varnish lines, as shown in Fig. 3, while the soluble portions have been completely removed from between the lines.

The dot pattern, which contains mercurous chloride may then be developed to visibility, as shown in Fig. 4, by means of a chemical developer comprised of the following:

|          | Parts |
|----------|-------|
| Water    | 100   |
| Thiourea | 1.7   |

The developer does not affect the portions of the lines 3 between the dots, so that the developed pattern appears as a relatively light tone, useful for light tone effects in the drawing which will ultimately be used for camera copy.

The line pattern which contains both mercurous chloride and basic lead sulphate may then be developed to visibility, as shown in Fig. 5, by means of a chemical developer composed of the following:

|                 | Parts |
|-----------------|-------|
| Water           | 100   |
| Sodium sulphide | 5     |

This developer affects both the dots and the portions of the lines 4 between the dots, so that the developed pattern appears as a relatively dark tone useful for dark tone effects in the drawing which will ultimately be used for camera copy.

The sheet, after the final washing referred to above, is suitable for use, but the surface is not one that will readily accept the chemical developer to which reference has been made or india drawing ink, with which the line drawings are usually made. It can be improved in this respect by the application of a suitable surface coating. Such a coating can be prepared as follows:

|               | Parts |
|---------------|-------|
| Water         | 1000  |
| Corn starch   | 60    |
| Gelatin (dry) | 50    |

Soak one half hour and with stirring melt to 120° F.

Add slowly with stirring 700 parts isopropyl alcohol.

Just prior to coating add 5 parts formalin.

Keep solution at 80° F. while coating and apply

on a regular engraver's plate coating machine for good uniformity of coating thickness.

For some purposes, particularly that described in the copending application of Louis S. Sanders, Serial No. 451,700, it is desirable to have a medium of the character described, on a transparent base, rather than on paper. For such purposes, it is only necessary to print the patterns on heavy weight sheet material of cellulose acetate, cellulose nitrate, or ethyl cellulose. Material of a thickness ranging from .003" to .010" is suitable. With such a material as a base the preparation of the drawing medium is essentially the same as that described above in connection with the preparation of the paper base medium.

It will be apparent from the foregoing that by forming patterns of intersecting lines, perfect registry or proper relative location between the patterns is readily obtained, without the necessity of taking any undue precautions during the imprinting of the patterns.

It will also be apparent that in cases where a transparent base is employed, the medium is especially useful in multi-color work, since the light pattern or tone is available to indicate a light shade of a selected color, and the dark pattern or tone is available to indicate a darker shade of said color.

As a modification of the invention, instead of using waterproof coated or laminated paper as the base of the medium, a gelatin coated paper sheet may be used, such for example, as imbibition paper furnished by Eastman Kodak Company. This is a hard smooth coated paper bearing a surface of plain hardened gelatin.

Using the same line printing plate as already described, there is imprinted upon this gelatin-surfaced paper a first pattern with a waterproof printing varnish or ink. This varnish imprint, consisting of the lines 10 in Fig. 6, is permitted to dry and then crossed, as in the previously described method, with a line print of mercurous chloride ink. In this instance, the mercurous chloride ink adheres permanently to the gelatin surface between the varnish lines as well as to the lines themselves, and is shown as the lines 11 in Fig. 7.

After the mercurous chloride ink has been permitted to dry the sheet is immersed for about 30 seconds in a solution containing

|                       | Parts |
|-----------------------|-------|
| Water                 | 100   |
| Lead acetate (normal) | 5     |

The excess of this solution is removed by rollers or blotting, and the sheet is then immersed for five or ten seconds in a solution containing

|                             | Parts |
|-----------------------------|-------|
| Water                       | 100   |
| Sodium sulphate (anhydrous) | 8     |

This operation produces an insoluble precipitate of lead sulphate within the gelatin surface between the varnish lines at the points 12 (Fig. 7), which lines serve as a resist to the lead acetate and sodium sulphate solutions.

After the sheet has become thoroughly dry, it is immersed in a solvent for the varnish lines, and with slight sponging or brushing, they are completely removed. There is a great number of varnish solvents, but it has been found that ethylene glycol monomethyl ether is particularly suitable, since it has low flammability and is non-toxic.

Removal of the varnish lines also removes the superimposed mercurous chloride ink and leaves

only the ink which adhered to the gelatin surface between the lines 10. This remaining mercurous chloride ink is in the form of isolated squares and constitutes the dot pattern. The lead sulphate also remains as squares alternating with the mercurous chloride squares. Together, these form continuous lines, as shown in Fig. 8, and by joint development, form the line pattern.

The mercurous chloride squares may be developed, as indicated in Fig. 9, by means of the thiourea solution which has been previously described. The mercurous chloride and lead sulphate squares may be collectively or simultaneously developed, as indicated in Fig. 10, by means of the sodium sulphide solution which has previously been described.

In this modified method of forming the medium, other chemicals may be substituted for the lead sulphate, such as cobaltous phosphate, nickelous phosphate, cupric tungstate, ferric phosphate, thallium tungstate or other insoluble metal salts which will produce non-actinic colored precipitates with a soluble sulphide, such as the sodium sulphide solution to which reference has been made.

With further reference to the modified method of forming the medium, it will be understood that while the method has been described in connection with gelatin-coated paper, that a transparent medium can be formed in the same manner, by starting with a transparent base sheet, as described in connection with the first form of the invention, and applying a coating of gelatin to such a base sheet. In this way, the medium thus prepared is suitable for multicolor work.

I claim:

1. In a method of preparing a medium for use in making camera copy, the steps which consist in imprinting upon a surface a pattern consisting of spaced parallel lines of a tacky substance, dusting said surface with basic lead sulphate to thereby cause said sulphate to adhere to said lines, removing said sulphate from the other portions of said surface, imprinting said surface with spaced parallel lines extending angularly to said first-named lines and by means of an ink containing mercurous chloride, and then removing said ink from all portions of said surface except at the points where the ink is superimposed on said first-named lines.

2. A method, as defined in claim 1, in which the surface, as a final step, is covered with a coating which improves the ability of the surface to accept chemical developers and drawing ink.

3. In a method of preparing a medium for use in making camera copy, the steps which consist in imprinting upon a surface a series of spaced parallel lines of a waterproof substance, then imprinting said surface with spaced parallel lines extending angularly to said first-named lines, and containing a chemically-developable material, and then applying a chemically-developable material, other than said first-named material, to the spaces enclosed by said lines.

4. In a method of preparing a medium for use in making camera copy, the steps which consist in imprinting upon a gelatin-coated surface a series of parallel lines of a waterproof substance, then imprinting said surface with spaced parallel lines extending angularly to said first-named lines, and containing mercurous chloride, then applying a chemically-developable material, other than mercurous chloride, to the spaces enclosed by the lines, and then removing said first-named lines from said surface.

5. In a method of preparing a medium for use in making camera copy, the steps which consist in imprinting upon a gelatin-coated surface a series of parallel lines of a varnish, then imprinting said surface with spaced parallel lines extending angularly to said first-named lines, and containing mercurous chloride, then immersing said surface in chemicals whose reaction produces an insoluble precipitate of lead sulphate in the spaces enclosed by said lines, and then removing said varnish lines by means of a suitable solvent.

6. In a method of preparing a medium for use in making camera copy, the steps which consist in imprinting upon a gelatin-coated surface a series of parallel lines of a waterproof varnish, then imprinting said surface with spaced parallel lines extending angularly to said first-named lines, and containing mercurous chloride, then successively immersing said surface in solutions of lead acetate and lead sulphate, whereby to form an insoluble precipitate of lead sulphate in the spaces enclosed by said lines, the varnish lines serving as a resist to said solutions, and then dissolving and removing the varnish lines from said surface.

7. A medium for use in preparing camera copy, said medium consisting of a surface having chemically-developable patterns thereon, said patterns consisting of spaced parallel continuous rows of contiguous segmental pattern areas, alternate segmental pattern areas of said rows being developable by one chemical to form a dot pattern and said rows in their entirety being developable by means of another chemical said rows of segmental pattern areas being separated by portions of said surface which are nonresponsive chemically to either of said chemicals.

8. A medium for use in preparing camera copy, said medium consisting of a surface having chemically-developable patterns thereon, said patterns consisting of spaced parallel continuous rows of contiguous segmental pattern areas alternate segmental areas in said rows containing lead sulphate and the remaining areas of said lines containing mercurous chloride whereby said segmental areas may be selectively chemically developed to provide visible dot patterns of different densities, said rows of segmental pattern areas being separated by portions of said surface which are nonresponsive chemically to developers of either of said chemicals.

9. A medium for use in preparing camera copy, said medium consisting of a gelatin-coated sheet, the surface of which bears chemically-developable patterns, said patterns consisting of spaced parallel continuous lines, uniformly spaced sections of which contain a chemically-developable material, and the sections of which intermediate said spaced sections contain a chemically-developable material other than said first-named material.

10. In a method of printing camera copy the steps of forming on a surface with chemically-developable photographically invisible material a Mosaic pattern of segmental pattern areas, certain of which areas being rendered visible in response to treatment by one chemical developer and others of said segmental pattern areas being rendered visible in response to treatment by another chemical developer, said segmental areas being contiguous and aligned in parallel rows, removing all trace of pattern material between said rows, and then selectively developing the segmental areas to form a visible dot pattern.